

## UNITED STATES PATENT OFFICE.

GILBERT MICHEL, OF BAGNEUX, FRANCE.

## PROCESS FOR THE PROTECTION OF THE SURFACE OF BATHS OF EASILY-OXIDIZABLE METALS SUCH AS MAGNESIUM.

No Drawing. Application filed August 2, 1926, Serial No. 126,727, and in France August 18, 1925.

Application for French patent has been filed on Aug. 18, 1925, and for British patent has been filed on Feb. 10, 1926.

The present invention has for its object a process for the protection of the surface of baths of easily oxidizable metals consisting essentially in distributing sulphur, not directly upon the metallic surface, but upon a layer of a protective substance which itself forms a protecting crust, such for instance as the fluoride of the metal under consideration.

It thus embraces the employment of magnesium fluoride for forming the protective crust on a bath of molten magnesium.

The invention may be carried into effect by way of example in the following manner in the case of molten magnesium.

A protective crust of magnesium fluoride is formed on the surface of the molten metal. This constitutes a solid crust which floats on the surface and constitutes in itself a good protection for the metal.

Pulverulent sulphur is then sprinkled upon the protecting layer where it melts and burns slowly, since the crust of fluoride has a much lower temperature than the molten metal and obviously the crust is not a good conductor of heat.

On account of this the evolution of sulphurous gas becomes so slow that the operator is not incommoded thereby and, in addition, direct contact of the sulphur with the metal being avoided, the formation of sulphides and oxy-sulphides need not be feared.

It must be understood that the protective layer of magnesium fluoride may be replaced by other fluorides or even chlorides. It may,

for example, consist of ammonium chloride alone or in combination with magnesium fluoride, but magnesium fluoride presents the advantage of avoiding the introduction of new impurities into the bath, such as, for example chlorides of magnesium. Magnesium fluoride constitutes an effective purifying agent for magnesium (as covered in my co-pending application, Ser. No. 7,156, Feb. 5, 1925). A chloride (e. g.  $MgCl_2$ ) would not have this effect, but would introduce chloride into the metal.

It is to be understood that the present invention covers the use of fluoride of magnesium in the form of a crust for the protection of light metals, both with and without the creation of a neutral surrounding atmosphere by the addition of sulphur.

I claim:

1. A method of protecting the surface of a bath of easily oxidizable metal which consists in covering the free surface of the bath with a protective layer and covering the crust so formed with sulphur.

2. A method of protecting the surface of a bath of easily oxidizable metal which consists in covering the free surface of the bath with a protective layer of the fluoride of the said metal and covering the crust so formed with sulphur.

3. A method of protecting the surface of a bath of molten magnesium, which consists in covering the free surface of the bath with a protective layer of magnesium fluoride, and covering the crust so formed with sulphur.

In testimony whereof I affix my signature.

GILBERT MICHEL.